

May 19, 1953

J. E. BAXTER

2,639,245

SULFIDE COATING

Filed Jan. 12, 1950

EFFECT OF VARIOUS ANIONS IN TERMS OF MINIMUM TEMPERATURE REQUIRED  
TO PRODUCE A COATING ON A STAINLESS STEEL IN 3 MINUTES.



INVENTOR.  
John E. Baxter.

BY

Harness, Dickey & Pierce.

ATTORNEYS.

## UNITED STATES PATENT OFFICE

2,639,245

## SULFIDE COATING

John Edgar Baxter, Detroit, Mich., assignor to  
 Parker Rust Proof Company, Detroit, Mich., a  
 corporation of Michigan

Application January 12, 1950, Serial No. 138,251

12 Claims. (Cl. 148—6.24)

1

This invention concerns a composition and method for the forming of sulfide coating on a steel surface; particularly on corrosion resistant and stainless steel surfaces.

It is known that acid solutions of sulfites and certain other sulfur compounds can be used to attack the surface of a ferrous metal to form a sulfide coating thereon. These coatings may serve various functions. For example, in some cases they are used as a paint base and in some cases they are used as a protective coating for the metal when the latter is subjected to wear or to extensive plastic deformation as in drawing and the like. The coatings, because of their insolubility in acid solutions, are superior to phosphate and oxalate coatings in those uses which require contact of the coating with oils of high acidity.

In order to form such a coating it is necessary that the solution attack the surface of the metal and form a salt of the metal. It has been pointed out, however, that the acid should not be sufficiently strong to cause excessive pickling of the metal since such pickling action, if too energetic, will prevent the forming of a coating. Therefore, it has been the practice to limit the acidity of the solution and to increase the rate of attack of the solution on the metal to the point desired by a suitable increase in the solution temperature.

The problem of securing both adequate and a controllable attack of the acid on the metal surface has been accentuated in the case of stainless steels which are normally quite resistant to acid attack. The forming of sulfide coatings on such normally resistant metal surfaces is usually carried out at temperatures near the boiling point of water, and, at best, in the range of 170–200° F. Therefore, the process has been subject to all the disadvantages of high temperature operation; particularly the high vapor pressure of the treating solution and the difficulty of handling acid solutions at such temperatures.

It is an object of this invention to provide a solution and a method for the forming of a sulfide coating on the surface of a steel object, particularly on a corrosion resistant or on a stainless steel object.

A further object is to provide a strongly acid composition for the treatment of a steel surface to form a sulfide coating thereon while avoiding the excessive pickling effect normally encountered with such compositions.

It is a still further object to form a sulfide coating on a steel surface, particularly corrosion resistant and stainless steel surfaces, at temperatures much lower than those used heretofore.

I have now found that the foregoing and related objects can be secured by subjecting the

2

surface of the steel to the action of an acidic aqueous solution comprising as essential ingredients the sulfide ion or compounds capable of yielding the sulfide ion at said steel surface; an anion of the group consisting of chloride, bromide, iodide, and thiocyanate; and a proportion of an acid sufficient to provide a pH below about 1.1.

Preferred compositions include the sulfite ion; but sulfide, thiosulfate, reducible organic sulfur-containing ions, etc., may be used. All such ions, other than the sulfide ion itself, form sulfide ions at the metal surface through reduction by the metal.

The drawing illustrates graphically the effect of the added anion in lowering the temperature required to produce a satisfactory coating on an 18-8 stainless steel in an arbitrarily selected short period of time. The time chosen is three minutes. The curves labeled A, B, and C represent additions of bromide, chloride, and iodide ions respectively to a 5% nitric acid solution containing 0.32% sulfite ion. The curve labeled D represents the addition of thiocyanate ion to a 5% sulfuric acid solution containing 0.32% sulfite ion.

As shown in the graphs, a 5% nitric acid solution containing 0.32% sulfite ion is capable of producing a suitable coating at about 172° F. in three minutes. The addition of even minor proportions of the added anions effects a marked reduction in the temperature required to produce such a three-minute coating. As shown in the graph, a 5% sulfuric acid solution containing 0.32% sulfite ion produces a satisfactory three-minute coating at about 165° F. Similarly, very small proportions of thiocyanate ion effect a marked reduction in the temperature required for such a three-minute coating.

Each of the curves depicted was determined by a large number of individual determinations and is typical of those obtained with a variety of acids and a variety of sulfide ion producing materials.

I have found that two limitations, that is, the degree of acidity and the presence of the added anion, are necessary to the obtaining of a successful result. If the pH of the solution is higher than about 1.1 the addition of the anion has little advantage. Where, however, the pH of the solution is less than about 1.1 even very small percentages of the added anion have a marked effect, especially in the lowering of the temperature required for the formation of an effective coating in a reasonably short time. For example, as little as 0.1 percent chloride has a marked effect on the temperature required where the pH is less than 1.1.

The lower limit of pH is not critical and de-

pends somewhat on the particular acid chosen, the concentration of the added anion, the degree of pickling action produced, the particular steel being coated and the degree of pickling which can be tolerated for the type of coating desired. However, it may be stated as a general rule that the pH range to be used is from 0.3 to 1.1. No particular advantage is gained by operating at the extreme limits of acid concentration since the entire advantage of the invention can be obtained when the pH is less than 1.1 and substantially above 0.5. If, however, it be desired to operate at the lowest possible pH, it is a matter of a few simple tests to establish the lower limit permissible with the particular steel and the particular anion which it is desired to use.

The sulfite ion concentration is normally maintained at about 0.3 to 1.3% but this proportion has been varied over relatively wide limits. It is preferred that the chloride ion or equivalent anion be maintained above about 1% in order to secure the maximum benefits from the invention, but some advantage can be gained with very minor percentages. Highly concentrated solutions, up to saturation, of the various anions can be used but little advantage is gained above 1.3% sulfite or about 5% of the activating anion.

Since hydrochloric acid is a source of both acid and chloride ion it may be the sole added agent, its minimum concentration being determined by the pH of the solution. Similarly, and where a small percentage of chloride ion is desired, hydrochloric acid may be used as a source of chloride ion and a second acid may be added to adjust the solution to the acidity desired. The proportion of hydrochloric acid required to produce a pH below 1.1 will provide a chloride percentage in excess of about 0.4%. Thus, for example, a solution containing less than about 0.4% can be made by using a limited proportion of hydrochloric acid and acidifying the solution to a pH below 1.1 with a second acid.

The particular acid selected is not important except that it be strong enough to provide the required pH. The mineral acids are both stronger and inexpensive as compared with other acids, e. g., benzene sulfonic and trichloroacetic, and hence are preferred. Sulfuric, hydrochloric, and nitric acids are especially preferred. Acids, which are not sufficiently strong to give the desired pH may be used if a suitable proportion of a stronger acid is used in the same composition. Similarly the source of sulfite, chloride, etc., is not important provided the cation provided with said anion be compatible with the solution; that is, not precipitate out an essential ingredient or have any other adverse effect on the solution or the coating.

The metals treated comprise the entire category of steels including mild steels, corrosion resistant, and stainless steels and, as pointed out previously, the invention has particular advantage in treating stainless steels because of the avoidance of the high temperatures normally required in their coating. The coatings produced are salts of the metals treated and vary somewhat with different alloys. Certain of the metals encountered in alloy steels have a tendency to form an oxide rather than a sulfide and, therefore, the average coating contains some oxide. Nickel appears to be particularly active toward the compositions of the invention

and nickel steels usually produce a high percentage of nickel sulfide in the coating.

The following examples illustrate the borderline conditions where the anion is deficient (Example 1); the acid is deficient (Example 2); and the acid and anion are both sufficient but at a relatively low concentration (Example 3). Example 4 illustrates the effects of increasing percentages of chloride ion on the lowering of the temperature required to obtain a satisfactory coating in three minutes. Three minutes has been chosen as a standard of comparison in the various examples. An 18-8 stainless steel was used in each example to give comparative results.

#### Example 1

A solution was made up containing 10 grams of sodium sulfite per gallon of water and containing 20 cc. of 95% sulfuric acid. The solution had a pH of 1.1. A temperature of 200° F. was required to produce a coating on the stainless steel in three minutes.

#### Example 2

A solution similar to that of Example 1 was prepared except that 20 cc. of 36% hydrochloric acid solution was used in place of the sulfuric acid. This produced a solution with a pH of 1.5 and a chloride content of 0.2%. Fifteen minutes were required at 200° F. to produce a coating on the stainless steel.

#### Example 3

The proportion of acid in Example 2 was doubled. This produced a solution with a pH of 1.1 and a chloride content of 0.4%. A good coating was produced in three minutes at 130° F.

#### Example 4

A series of solutions containing 5% nitric acid and 0.32% sulfite as sodium sulfite was made up. Each of the solutions contained successively the following chloride percentages: 0.0, 0.1, 0.2, 0.3, 0.5, and 5.0%. In the solution containing no chloride a coating was produced in 3 minutes at 172° F. and no coating could be produced at 170° F. In the remaining solutions containing from 0.1 to 5% chloride a satisfactory coating was obtained in three minutes at 150°, 146°, 142°, 140°, and 100° F. respectively.

Although I do not wish to be limited by theory, I believe that the chloride ion, or equivalent anion, has an activating influence on the acid attack on the metal. This permits a suitable and controlled attack at a lower temperature for the purpose of forming a coating on the metal. It appears also that the activation does not significantly increase the pickling effect, but, in some cases, may reduce this effect when full advantage is taken of the lowered coating temperature. As indicated previously, the invention permits of a more rapid coating of stainless and corrosion resistant steels and is particularly advantageous in this respect.

I claim:

1. A composition for forming a sulfide coating on a steel surface which consists of an aqueous solution of a member of the group consisting of the sulfide ion and ions which form the sulfide ion through reduction on the steel surface and in a proportion equivalent to about 0.3-1.3 percent sulfite ion; a member of the group of anions consisting of chloride, bromide, and iodide, in a proportion of from equivalent to .1% of the chloride ion up to and including saturation; and an acid

selected from the group consisting of sulfuric, hydrochloric, and nitric in a proportion sufficient to provide a pH in the range of about 0.3-1.1.

2. A composition for forming a sulfide coating on a steel surface which consists of an aqueous solution of a member of the group consisting of the sulfide ion and ions which form the sulfide ion through reduction on the steel surface and in a proportion equivalent to about 0.3-1.3 per cent sulfite ion; the chloride ion in a proportion of from .1% up to and including saturation; and an acid selected from the group consisting of sulfuric, hydrochloric, and nitric in a proportion sufficient to provide a pH in the range of about 0.3-1.1.

3. A composition for forming a sulfide coating on a steel surface which consists of an aqueous solution of a member of the group consisting of the sulfide ion and ions which form the sulfide ion through reduction on the steel surface and in a proportion equivalent to about 0.3-1.3 percent sulfite ion; the chloride ion in a proportion of from about 1% to about 5%; and an acid selected from the group consisting of sulfuric, hydrochloric, and nitric in a proportion sufficient to provide a pH in the range of about 0.3-1.1.

4. The method of forming a sulfide coating on a steel surface which comprises contacting the surface with an aqueous solution consisting of water, the sulfide ion and ions which form the sulfide ion through reduction on the steel surface and in a proportion equivalent to about 0.3-1.3 percent sulfite ion; a member of the group of anions consisting of chloride, bromide, and iodide, in a proportion of from equivalent to .1% of the chloride ion up to and including saturation; and an acid selected from the group consisting of sulfuric, hydrochloric, and nitric in a proportion sufficient to provide a pH in the range of about 0.3-1.1.

5. The method of forming a sulfide coating on a steel surface which comprises contacting the surface with an aqueous solution consisting of water, the sulfide ion and ions which form the sulfide ion through reduction on the steel surface and in a proportion equivalent to about 0.3-1.3 percent sulfite ion; the chloride ion in a proportion of from .1% up to and including saturation; and an acid selected from the group consisting of sulfuric, hydrochloric, and nitric in a proportion sufficient to provide a pH in the range of about 0.3-1.1.

6. The method of forming a sulfide coating on a steel surface which comprises contacting the surface with an aqueous solution consisting of water, the sulfide ion and ions which form the sulfide ion through reduction on the steel surface and in a proportion equivalent to about 0.3-1.3 percent sulfite ion; the chloride ion in a proportion of about 1% to about 5%; and an acid selected from the group consisting of sulfuric, hydrochloric, and nitric in a proportion sufficient to provide a pH in the range of about 0.3-1.1.

7. A composition for forming a sulfide coating on a steel surface which consists of an aqueous solution of a member of the group consisting of the sulfide ion and ions which form the sulfide ion through reduction on the steel surface and in a proportion equivalent to about 0.3-1.3% sulfite ion; a member of the group of anions consisting of chloride, bromide, and iodide in a proportion of about 1% to about 5%; and an acid selected from the group consisting of sulfuric, hydrochloric, and nitric in a proportion sufficient to provide a pH in the range of about 0.3-1.1.

8. The method of forming a sulfide coating on a steel surface which comprises contacting the surface with an aqueous solution consisting of water, the sulfide ion and ions which form the sulfide ion through reduction on the steel surface and in a proportion equivalent to about 0.3-1.3% sulfite ion; a member of the group of anions consisting of chloride, bromide, and iodide in a proportion of about 1% to about 5%; and an acid selected from the group consisting of sulfuric, hydrochloric and nitric in a proportion sufficient to provide a pH in the range of about 0.3-1.1.

9. A composition for forming a sulfide coating on a stainless steel surface which consists of an aqueous solution of a member of the group consisting of the sulfide ion and ions which form the sulfide ion through reduction on the steel surface and in a proportion equivalent to about .3 to 1.3% sulfite ion, the bromide ion in a proportion of from equivalent to .1% of the chloride ion up to and including saturation, and an acid selected from the group consisting of sulfuric, hydrochloric and nitric in a proportion sufficient to provide a pH in the range of about .3 to 1.1.

10. A composition for forming a sulfide coating on a stainless steel surface which consists of an aqueous solution of a member of the group consisting of the sulfide ion and ions which form the sulfide ion through reduction on the steel surface and in a proportion equivalent to about .3 to 1.3% sulfite ion, the iodide ion in a proportion of from equivalent to .1% of the chloride ion up to and including saturation, and an acid selected from the group consisting of sulfuric, hydrochloric and nitric in a proportion sufficient to provide a pH in the range of about .3 to 1.1.

11. The method of forming a sulfide coating on a steel surface which comprises contacting the surface with a solution consisting of water, the sulfide ion and ions which form the sulfide ion through reduction on the steel surface, and in a proportion equivalent to about .3 to 1.3% sulfite ion, the bromide ion in a proportion of from equivalent to .1% of the chloride ion up to and including saturation, and an acid selected from the group consisting of sulfuric, hydrochloric and nitric in a proportion sufficient to provide a pH in the range of about .3 to 1.1.

12. The method of forming a sulfide coating on a steel surface which comprises contacting the surface with a solution consisting of water, the sulfide ion and ions which form the sulfide ion through reduction on the steel surface, and in a proportion equivalent to about .3 to 1.3% sulfite ion, the iodide ion in a proportion of from .1% up to and including saturation, and an acid selected from the group consisting of sulfuric, hydrochloric and nitric in a proportion sufficient to provide a pH in the range of about .3 to 1.1.

60 JOHN EDGAR BAXTER.

References Cited in the file of this patent

UNITED STATES PATENTS

|    | Number    | Name            | Date          |
|----|-----------|-----------------|---------------|
| 65 | 2,273,234 | Tanner          | Feb. 17, 1942 |
|    | 2,301,983 | Tanner          | Nov. 17, 1942 |
|    | 2,302,643 | Thompson        | Nov. 17, 1942 |
|    | 2,314,565 | Thompson        | Mar. 23, 1943 |
| 70 | 2,550,660 | Amundsen et al. | May 1, 1951   |
|    | 2,577,887 | Gibson          | Dec. 11, 1951 |

FOREIGN PATENTS

|    | Number  | Country | Date          |
|----|---------|---------|---------------|
| 75 | 131,106 | Austria | Jan. 10, 1933 |